

Patented June 4, 1929.

## UNITED STATES PATENT OFFICE.

WILLIAM HOWARD COLE, OF PARIS, FRANCE.

## DERUSTING FERROUS METALS.

No Drawing. Original application filed September 20, 1927, Serial No. 220,840, and in Great Britain August 22, 1927. Divided and this application filed December 31, 1927. Serial No. 244,042.

This specification is a division of my specification Serial No. 220,840, filed 20th September, 1927.

I have found that by treating rusted iron or steel articles with dilute phosphoric acid, in an autoclave, at high temperature and pressure, the rust on the said article is removed.

The following example will further illustrate the nature of the invention.

A steel container with a manhole opening was made strong enough to withstand high pressure. This container was furnished with a pressure gauge, a safety valve and in addition a soft metal plug which would melt if the temperature rose too high, and so release the pressure, and finally a signal whistle which whistled an alarm when the pressure inside rose to the predetermined point. This whistle alarm was made to be adjustable for any pressure wanted. In one experiment, after introducing the ingredients and steel and iron pieces to be de-rusted, the pressure arranged for was about 50 pounds per square inch, the heating had only to be used for a period of about ten minutes before the whistle gave the alarm and the source of heat was turned off. After the pressure vessel had cooled sufficiently to enable it to be opened without danger, which in this case was about 10 minutes, the autoclave was opened and it was ascertained that the iron and steel pieces treated were in

appearance very clean and free from rust. I do not confine myself to the use of dilute phosphoric acid for de-rusting as described above, as I find that my high pressure process gives excellent results with other ingredients, for the compositions of which I do not claim priority, but merely desire, in this respect, to be protected in the use of my hereinbefore described method of treatment under pressure and high temperature, and the use of an autoclave or closed vessel capable of withstanding heat and pressure for rust-proofing and de-rusting ferrous metals.

What I claim and desire to secure by Letters Patent is:—

1. Process of de-rusting and removing scale from ferrous articles consisting in treating them with phosphoric acid so dilute that no coating is left on the articles treated in a closed vessel, said treatment being carried out at boiling temperature and under pressure greater than atmospheric pressure.

2. Process of de-rusting and removing scale from ferrous articles consisting in treating them with phosphoric acid so dilute that no coating is left on the articles treated in a closed vessel, said treatment being carried out at a boiling temperature and under a pressure of about 50 pounds per square inch.

In testimony whereof I affix my signature.

WILLIAM HOWARD COLE.